

## UNITED STATES PATENT OFFICE.

WILLIAM S. GOULD, OF NEW YORK, AND WILLARD B. OSBORNE, OF ELMA, NEW YORK,  
ASSIGNORS TO GOULD STORAGE BATTERY COMPANY, INC., OF NEW YORK, N. Y., A  
CORPORATION OF NEW YORK.

## SEPARATOR AND METHOD OF MAKING THE SAME.

No Drawing.

Application filed October 23, 1923. Serial No. 670,322.

Our invention relates to storage battery separators and method of making the same. It has long been the desire of storage battery manufacturers to produce a battery with treated separators which can be shipped dry. The difficulty heretofore experienced has been that if the treated separators were dried before placing in the battery they split or curl to such an extent that they are destroyed or greatly injured in the assembly of the battery elements. If such separators are placed in the battery in a damp condition, the action is detrimental to the positive plates. So far, no method has been devised whereby the separators, after treatment with the usual alkali treatment, could be sufficiently dried for assembly in the battery. Such separators as heretofore manufactured must be kept wet or damp until placed in the battery in order to avoid destructive curling, splitting and cracking.

We have devised a method of treating the separators whereby they may be completely dried without any curling, cracking or splitting. By reason of this method, the battery elements may be assembled dry in the factory, shipped to their destination and the electrolyte supplied, thus avoiding the dangers and other difficulties of transporting a battery containing sulphuric acid electrolyte. Furthermore, the separators resulting from our method may be stored by manufacturers and dealers in a dry state, thus greatly simplifying the problem of carrying a stock of separators. It has heretofore been necessary to keep such separators in large tanks where they could be kept wet until used.

A suitable wood, such as Port Orford white cedar in the form of boards or veneer are put into a solution of approximately 3% caustic soda at a temperature at approximately 212° F. for about eight hours. They are then removed from this solution and placed in clear running water for about fourteen hours to remove the caustic soda. They are then put into a weak solution of sulphuric acid about 1.02 specific gravity and left there a sufficient time to allow the sulphuric acid to neutralize any caustic soda that might remain in the wood after washing, usually about two hours. They are then immersed in hot water for about two

hours which neutralizes the acid. They are then put through a drying machine of any desired construction but preferably having a series of movable steam-heated, horizontal, iron plates, which rest against the opposite surfaces of the boards or veneer and which iron plates are heated sufficiently to rapidly dry the wood. The plates hold the wood flat while it is being dried and preferably are so arranged that the wood is held under a slight pressure between the hot plates. As a result of this drying step, the wood boards or veneer are thoroughly dried and held against curling or splitting. After the stock is thus treated and dried it is then grooved and cut to the desired lengths in the ordinary way to form separators of the required size and thickness. Such separators possess their natural porosity, permeability and cellular structure and mechanical strength. These separators may be stored, handled and otherwise used in the same manner as untreated wood separators.

While we prefer to dry the stock while confined between heated plates, the stock may be dried by hanging it in a drying room after it has been treated by the alkali process, but before the stock has been cut into separators. In this instance, some of the stock will be wasted because cracks develop at the ends of the stock during the drying step and it is, therefore, necessary to remove the cracked portions from the stock after it is dried and before the separators are cut.

We do not intend that our invention shall be limited to any particular type of drying machine but have found that a machine, such as that generally used in the treating of wood veneer, is preferable.

While we do not fully understand the reasons why the separators, when treated, according to our method, do not curl, we are, of the opinion, that the cracking, curling and splitting are prevented by the pressure exerted upon the wood during the time that it is being dried in the machine. Also the curling is prevented because the heated plates hold the stock flat and dry the fibres while they are confined and while holding them against any tendency to warp or curl until they are completely dried and any tendency to warp or split is removed or neutralized.

In our opinion, the reason why the boards do not crack objectionably when dried in

a drying room is that, when this step is to be followed, the stock is cut slightly larger than necessary and because of the complete drying of the boards before they are cut into separators the outer portions of the stock act to limit the cracking and curling. It is to be understood when this method is pursued, an allowance must be made for certain waste both at the ends of the stock and also on the sides thereof. It is largely on this account that we prefer to use means for holding the stock while drying.

Many methods of alkali treatment may be applied to the separators and a great variety of machines may be used for drying the stock without departing from the spirit of our invention.

We claim:

- 20 1. The method which consists in treating a separator to remove such of its constituents as would deleteriously attack lead when subjected to electrolytic action and drying the separator between heated surfaces.
- 25 2. The method of treating separators which consists in subjecting the separators to a caustic soda treatment and drying them between heated surfaces.
- 30 3. The step in the treatment of separators which consists in drying said separators between heated surfaces after said separators

have been subjected to the action of an alkali.

4. The steps in the treatment of separators which consists in first subjecting said separators to the action of an alkali and thereafter in drying said separators while held between heated surfaces. 35

5. The steps in the treatment of separators which consists in first subjecting said separators to the action of an alkaline solution 40 and thereafter in drying said separators between heated surfaces until substantially dry.

6. The steps in the treatment of separators which consists in first subjecting said separators to the action of an alkali and thereafter in drying said separators between hot metal surfaces. 45

7. The method of making separators which consists in treating sheets of wood with an alkali, washing the sheets, drying 50 them between heated surfaces and cutting the separators from the sheets.

8. A dry flat wood separator that has been treated with an alkali to remove such of its constituents as would be deleterious when used as a battery separator, said separator possessing its natural porosity and strength. 55

WILLIAM S. GOULD.  
WILLARD B. OSBORNE.